

## UNITED STATES PATENT OFFICE

ALBERT C. FISCHER, OF CHICAGO, ILLINOIS, ASSIGNOR TO THE PHILIP CAREY  
MANUFACTURING COMPANY, A CORPORATION OF OHIO

## COMPOSITION OF MATTER

No Drawing. Application filed February 2, 1926, Serial No. 85,587. Renewed May 7, 1931.

My present invention relates in general to a composition material for use primarily as expansion-contraction joints for masonry construction, and especially road construction, and has particular reference to an improved filling and reenforcing medium which is incorporated with a compressible binding material to make up the finished product.

The composition of the material is such that it may be used for purposes other than expansion-contraction joint, and in this connection I would like to mention floor coverings, bridge flooring, crossing planks, insulating sheets and other analogous uses. However, since the material is primarily intended for expansion joint I will use this example in the following description.

Expansion-contraction joint material is usually produced in preformed strips, or else in what is known as poured joint. In the latter instance the space between the slabs or sections in a roadway, or similar construction, is filled by pouring the material after the same has been prepared for this purpose.

While my present invention is applicable to either a preformed joint or a poured joint I will ordinarily offer the same as a preformed product.

In reducing the invention to practice I first select a binding material suitable for the purpose, having the desired inherent qualities of a compressible mastic material, or a composition of matter having such qualities. More specifically I would prefer to use bituminous matter, particularly blown asphalt, the same being prepared in a manner already well known to the art, except as to certain detailed steps, which will be hereinafter mentioned.

A compressible binder alone is not all together satisfactory as an expansion-contraction joint, but I can supply the qualities which are lacking by incorporating a filler with the binder. I have found that a filler should be selected for the desirable properties that it will add to the composition as well as overcome the unsatisfactory qualities of the binder. With this end in view I have found that a most satisfactory filler consisting of Tampico fiber, which is a stiff, harsh, but

pliant and bristle-like fiber, which is sometimes used as a substitute for animal bristles, as for instance in the making of cheap brushes.

In using this fibrous material the same may be considerably dried out between the time it is harvested and mixed with the binder to produce the joints. Should it be found to be too dry after it has been stored for a while, it could be saturated with water, oil, or with any other substance to make it supple and pliable. This treatment may or may not be desirable, but if so, I would suggest that a saturating solution be selected that would readily volatilize, so that when the material is mixed with the asphalt when the asphalt is in a heated state the liquid will volatilize so as to leave the cellular structure of the filling material unfilled. This would be desirable so that advantage could be taken of the resilient and reinforcing qualities of the filler, which is one of the reasons that I use a filler, and is also a reason why I have selected this kind of vegetable fibre. As a secondary step in saturating the filling material I can mention the possibility of pressing a surplus of the saturating solution from the material prior to its incorporation with the binding material. Also, care should be taken to use a saturant that will volatilize at a low temperature, since the asphalt will not be very hot when the filling material is incorporated. The reason for this is that so long as I keep the asphalt in a plastic state it will not saturate the filler. Of course the asphalt will have to be warm enough so as to realize a thorough mixing of the filling material.

The proportion of filling material used would vary to a reasonable degree, for instance, I would never use more than fifty (50) per cent of the Tampico fiber by weight to fifty (50) per cent binder, and in most cases I would use as little as fifteen (15) per cent by weight of the Tampico fiber and eighty-five (85) per cent of the binder. I may also, if occasion demands, use a secondary filling medium in combination with the vegetable fiber referred to, such as, for instance, ordinary excelsior, animal fibre, such

as bristles, in fact various combinations, but in any event the idea is to use the plants referred to as the primary filling medium, so as to obtain distribution of a tangled mass 5 of fibers or the like, throughout the compressible binder. When I refer to this tangled mass I make it clearer by stating that due to the long and pliant nature of the fiber they will be interlocked with each other, 10 which condition is brought about still more during the mixing step.

As a further feature I can also use this filling material in the form of a matted or felted unfilled mass, that is to say, the material instead of being distributed throughout the binder could be felted or compressed 15 into a matted mass and enveloped in a compressible binder. When I refer to an unfilled filler or matted mass it should be understood to mean that the binding material 20 has not penetrated the cellular structure of the material, nor has it filled the orifices in the mass. The individual pieces in such a felted matted mass need not adhere one to the 25 other, but should it be desirable that they do so the mass could be treated with an adhesive, such as, sodium silicate. Regardless of the form in which the filling material is used the resultant product will always include a 30 binder with a filler of this material.

From the above it will readily be seen that with the use of very inexpensive material I am able to produce a most satisfactory expansion joint composition.

35 I claim:

1. A preformed expansion joint comprising a plastic boardlike strip of bituminous material reenforced by a tangled mass of relatively long, stiff, but pliant, bristle-like 40 vegetable fibers which are intermixed and distributed therethrough.

2. A preformed contractile and expandible constructional material comprising a plastic board-like strip of bituminous material reenforced by a tangled mass of relatively long, stiff, but pliant, bristle-like vegetable fibers which are intermixed and distributed therethrough.

3. A preformed contractile and expandible constructional material comprising a plastic board-like strip of bituminous material reenforced by a tangled mass of relatively long, stiff, but pliant, bristle-like vegetable fibers which are intermixed and distributed therethrough in an unpenetrated state.

4. A preformed contractile and expandible constructional material comprising a plastic board-like strip of bituminous material reenforced by a tangled mass of Tampico fibers which are intermixed and distributed therethru in an unpenetrated state.

5. A preformed contractile and expandible constructional material comprising a mixture of about eighty-five per cent by

weight of bituminous binder and about fifteen per cent by weight of Tampico fibers.

6. A preformed contractile and expandible constructional material comprising a mixture of bituminous binder and a tangled mass of relatively long, stiff, but pliant, 70 Tampico fibers.

7. Constructional material comprising a body of bituminous composition having Tampico fibres incorporated and distributed 75 therein to reenforce the body into a cohesive mass.

8. A preformed expansion joint strip comprising a body of bituminous composition having Tampico fibres incorporated and distributed therein to reenforce the body into a cohesive mass.

9. A preformed constructional material comprising a mixture of bituminous binder and a tangled mass of relatively long, stiff, 85 but pliant, Tampico fibers.

10. A preformed constructional material comprising a plastic board-like strip of bituminous material reenforced by a tangled mass of relatively long, stiff, but pliant 90 bristle-like fibers.

11. A preformed contractile and expandible construction material comprising a plastic board-like strip of bituminous material reenforced by a tangled mass of relatively long, stiff, but pliant bristle-like fibers, which 95 are intermixed and distributed therethrough.

Signed at Washington, D. C., this 1 day of February, 1926.

ALBERT C. FISCHER. 100

105

110

115

120

125

130